

Patented Oct. 28, 1924.

## UNITED STATES PATENT OFFICE.

CHARLES P. MADSEN, OF NEW YORK, N. Y., ASSIGNOR TO MADSENELL CORPORATION,  
OF NEW YORK, N. Y., A CORPORATION OF NEW YORK.

## PHONOGRAPH RECORD AND METHOD OF PRODUCING THE SAME.

No Drawing. Application filed June 14, 1920, Serial No. 388,897. Renewed January 21, 1924.

*To all whom it may concern:*

Be it known that I, CHARLES P. MADSEN, a citizen of the United States, and a resident of the city of New York, county and 5 State of New York, have invented an Improvement in Phonograph Records and Methods of Producing the Same, of which the following is a specification.

My invention relates to records, particularly sound records, and to methods of producing the same. It is an object of my invention to devise a superior form of record, particularly sound records, for use in phonographs and the like, which shall possess 10 many advantages, such as superior durability and playing properties, greater ease and economy in manufacture, and other advantages more fully pointed out hereinafter, over the ordinary stamped record now on 15 the market and made from various plastic compositions. These composition molded or stamped playing records are not only frail, and short-lived, but are comparatively poor copies of the original, and it has 20 hitherto been impossible to make a metal record which will be free from surface noises and withstand the action of the 25 needle.

By way of example, I shall describe in 30 the accompanying specification illustrative embodiments of the process and product of my invention, it being understood, however, that my invention is not limited to such 35 illustrative embodiments which are herein set forth for the purpose of illustration only.

I have discovered that an electrodeposited metal record, as a "nickel metal", or nickel alloy record, will, when properly made, have 40 a smoother surface than the ordinary stamped record and will withstand the action of the needle or diamond better. It is to be understood that by the term "nickel metals", I mean to designate either nickel, 45 or cobalt, or alloys containing substantial amounts of either nickel, or cobalt, or both of these metals. I have furthermore discovered a new process of producing such metal playing records, as well as superior 50 "masters", "mothers" and "stampers" now used in the art of stamping records, which are very much cheaper and are more faithful copies of the original wax master than any heretofore produced. I am therefore 55 enabled to make not only a practical metal

playing record of metal at a low cost but also improved "masters", "mothers" and "stampers" for making the usual molded or composition records.

In making these new metal playing records, I may use the usual or well-known means for the electrodeposition part of the process, but I find, in doing so, that it is difficult to control the hardness and soundness of the metal, and to avoid the difficulties of deposition, especially in the case of the "nickel metals", including the curling or cracking open of the deposit during deposition. I therefore prefer to use for making such players, "masters", "mothers" and "stampers", the process of electrodeposition disclosed in my applications, Ser. No. 254,793, filed September 19, 1918 and Ser. No. 292,793 filed April 26, 1919, and find by doing so that many new and unexpected 75 results of great theoretical interest and great practical value, are obtained.

It is impractical to make nickel "mothers", "masters" and "stampers" of "nickel metals" by the old electrodeposition processes. I 80 find that my new nickel, or the other "nickel metals" as disclosed in application, Ser. No. 292,794 filed April 26, 1919, made in accordance with the processes disclosed in my application, Ser. No. 254,792, filed September 85 19, 1918, and application, Ser. No. 292,793, filed April 26, 1919, is very well adapted for the purpose, and that many advantages, and useful and unexpected results are gained by so doing.

I shall, in the accompanying specification, illustrate one embodiment of my invention by way of example, using my new nickel made by means of one of my new processes of electrodeposition referred to above, it being understood, however, that my invention is not limited to the illustrative embodiments herein set forth for the purpose of illustration only.

Briefly described, one form of my electrodeposition methods which may be successfully employed in connection with the present invention, makes use of a nickel anode, which is substantially free from occluded or combined oxygen, chromium, 100 copper and silicon, and also substantially free from "passive" or insoluble portions. Such an anode contains amorphous carbon and may be prepared by melting nickel shot 105 in a reducing atmosphere, such as atmos- 110

phere of carbon monoxide, together with from about .5 to about 2 per cent of amorphous carbon. The mixture should be stirred occasionally in a molten condition 5 and kept molten for about one half to about one hour, care being taken that the temperature is not raised to such a point as to graphitize the amorphous carbon. In casting such anodes, care should also be taken 10 not to let the cast cool too rapidly since it is desirable to prevent the formation of comparatively large crystals, the anode being better in operation where it is of a fine crystalline structure, with the average 15 longest dimension of the crystals being approximately between one-sixty-fourth and one sixteenth of an inch.

While various electrodeposition baths may be used in connection with the present invention, I prefer to use a bath made up of 20 nickel chloride ( $NiCl_2$ ), nickel sulphate ( $NiSO_4$ ), boric acid and a slight amount of sodium sulphate. The bath is preferably heated to a temperature of  $130^{\circ} F$ . In order 25 to deposit perfect metal, by which I mean metal which is sound, reguline, malleable and ductile and substantially free from pores, pits and hydrogen, the bath should have a very slight H-ion concentration of a 30 nickel solvent-acid, such as hydrochloric or sulphuric acid. The H-ion concentration should not, however, be great enough to cause substantial hydrogen evolution at the cathode. The bath should also have suspended therein finely divided or colloidal 35 "nickel metal" hydrate, such as nickelous hydrate.

By selecting a proper ratio between the area of the surface of the anode and the area 40 of the surface of the cathode, it will be possible to maintain the initial solvent-acid H-ion concentration of the bath through a considerable period of operation. This ratio may readily be determined by trial and 45 should be such as to cause a slight alkaline-tending characteristic to generate a slight amount of "nickel metal", as nickelous, hydrate, continuously during deposition.

Applying the electrodeposition process 50 just described to the present invention, I may prepare a wax master record in the usual manner. I may then for the purpose of making players first make by the usual and well-known means a copper metal 55 "master" by electrodeposition upon the wax "master", and I may treat this copper "master" for receiving a non-adhering deposit in the old way, as by sulphiding or silvering and then iodizing, and upon this 60 deposite my nickel players. I may also from this copper "master" make a copper "mother", and then treat this "mother" for receiving a non-adhering deposit, and from this make a "sub-master" or "stamper" upon 65 which I may deposit my metal player.

I may also make my metal "master" of "nickel metal" by deposition upon the wax "master", but I find this difficult to do because of the low softening point of the wax. I therefore prefer in making my new 70 "nickel metal" "mothers", "stampers" and playing records first to make a copper "master" upon the wax in the usual way. I then give this an extremely thin coating of my new "nickel metal", by any of my 75 new electrodeposition processes referred to above. A new and valuable result is obtained by so doing. This coating is not like the ordinary nickel plating in that it is impervious, free from hydrogen, and remarkably smooth. I find that a coating as thin as .00005 of an inch is impervious and can receive subsequent treatment without affecting the copper underneath and that this 80 thickness alters the dimensions of the sound record less than the usual sulphide or iodized silver coating formerly used.

I have discovered that treating the nickel surface as an anode in an electrolytic cell containing strong as 15 per cent solution 90 of sodium hydroxide or other alkali, with a current density of about 50 amperes per square foot for about two seconds, renders the "nickel metal" surface of the master or other record capable of receiving a freely 95 separable non-adherent coating of "nickel metal".

No visible change can be detected in the "nickel metal" surface as a result of this treatment and a microscopic examination 100 shows practically no increase or decrease in the size of the sound record grooves. This separation treatment is an improvement over the old means used for such purpose not only because it results in a more faithful reproduction 105 but also because the treatment is semi-permanent and one treatment will permit of many separable deposits being made in succession. Furthermore, the deposit made upon such a surface is much more easily 110 separable than by any now known treatment. I am, accordingly, enabled to make "nickel metal" deposits upon "nickel metal" surfaces treated by this method as thin as .0005" and remove them readily and perfectly, for use as "mothers", "stampers", "players", or for other purposes. By so doing not only are more faithful copies obtained, but they can be made very much thinner.

I therefore prefer to make my new metal player by depositing "nickel metal" upon the copper "master" coated with a thin layer of my new "nickel metal," and treat it with the separation process described above. In 125 commercial production, however, I prefer to use such a master for making a nickel "mother". Instead, however, of making this nickel "mother" of the same thickness as is necessary in making them in copper by the old 130

means referred to above, I find it necessary to make it only from .005 to .01 inch thick, and I find it will answer all purposes if made only .005 inch thick and is then afterwards reinforced with a waterproof paper cemented to its back, or by other suitable means. I may by this means make several such "mothers" from the "master," and from each of these make, by the same process, a number of "nickel metal" "sub-masters" or "stampers." These "sub-master" or "stampers" may be deposited to a thickness of about .020 inch and used as stampers for producing the usual molded or composition records. I find that such a stamper is far more durable than the usual copper stamper and that the molded records made from it are much more faithful copies of the original wax "master." The combination of these processes furthermore results in the saving of a great deal of time in the production of stampers, as I am enabled to turn out by this means the first stamper within about three days as against an average of 23 to 30 days by the old means, where the entire process is carried out in copper.

In using these "sub-masters" for making my new metal playing record, I find it is necessary to have them no thicker than .005 inch and if backed up with a waterproof paper, as described above, a thickness of only .0005 is necessary. Such a "sub-master" can, by my new process of deposition referred to above, be made in 5 minutes as against 48 hours in making a copper stamper by present means.

I may deposit these new playing records sufficiently thick to remain flat during playing and to withstand handling, which thickness I find in general to be .016 to .02 inch or I may deposit them only .0005 to .001 inch thick and back them up by electrodeposition or otherwise with another metal, as iron; or I may also back up a thin deposited sound record by uniting it with another metal plate, as iron, by means of soft or hard solder.

It is also obvious that whether the playing record consists of "nickel metal" only or whether it is backed up with another metal by electrodeposition or otherwise, two of them may be united back to back, either by means of soft or hard solder, or by a cement, or otherwise, and also in the case of uniting relatively thin playing records with a metal plate, as by hard or soft solder, one may be mounted on each side of the same plate.

I prefer, however, to make my new "nickel metal" or nickel alloy playing records comparatively thin, as say about .0005 to about .005 inch thick and to fasten them either with or without other electrodeposition or other metal backing, as iron, on a filler disc of one or more layers of tough resilient material, as plain or impregnated paper, cardboard, wood, bakelite paper, or other com-

position. I may cement the two deposited playing records back to back on one such layer, but in general I prefer to cement each player to a separate backing layer or backing, then dry the same, and unite these two, preferably under pressure in a vacuum dryer. For this purpose, I may use a cement consisting essentially either of waterproof glue, dextrin, casein, or water glass, but I prefer in general to add an inert filler as fine silica, or pulverized asbestos. I may, however, also cement these records to their backings with a heat-setting cement, as asphaltum, mastic or bakelite.

I find that this type of mounting for my new metal playing records results in many advantages. Although extremely light, they are amazingly strong and in fact almost unbreakable. The filler can be made with a degree of resiliency which will absorb considerable shock without injuring the sound groove, but sufficiently rigid to properly operate the sound producing mechanisms.

While I find that the new "nickel metal" made by my process referred to above, is sufficiently hard to withstand the needle action in reproducers of ordinary weight of from about three to about four ounces, I may make a nickel alloy metal player which is harder for heavier reproducers and for so-called "diamond" reproducers for "hill and dale" records.

I find that I can increase the hardness of my new electrodeposited nickel by slightly increasing the free solvent H-ion concentration of the bath so as to evolve a predetermined amount of free hydrogen at the cathode, and by means of my new anodes maintain this exact predetermined H-ion concentration necessary for this result, and thereby continuously produce a "nickel metal" deposit containing a definite amount of hydrogen sufficient to harden the "nickel metal" but not sufficient to cause it to curl or crack, which amount is in general from about one to five volumes of hydrogen per volume of electrodeposited "nickel metal."

I may also make an alloy deposit by depositing simultaneously two different metals from the same bath, as for instance, nickel and iron, or nickel and cobalt. I find that an electrodeposited alloy containing about 80% nickel and 20% cobalt is very hard. This alloy may be deposited from a bath of the same H-ion concentration as for nickel, and therefore may be made either hydrogen-free or with a controlled amount of hydrogen. In order to deposit a nickel-iron alloy, however, the solvent hydrogen-ion concentration must be such that an appreciable amount of hydrogen will be evolved at the cathode and absorbed by it. Such an alloy will always contain some hydrogen. In general, I find that an electrodeposited alloy of nickel with from about 1% to about

5% of iron and from one to five volumes of hydrogen is sufficiently hard.

I may also harden the surface of a "nickel metal" or metal alloy player by either sulphiding or oxidizing its surface, as by either treating it as an anode in an electrolytic cell containing an alkaline sulphide or hydroxide, or by heating it to a high temperature in air or in hydrogen sulphide. I find that the sulphides or oxides of nickel, for example, so formed are extremely hard and possess a glass-like smoothness. The nickel oxide formed is particularly smooth and many times harder than nickel and in fact almost approaching the hardness of carbonium.

For uses, however, where metal alloy playing records are desired, I may make them by depositing alternate layers of different metals in separate baths, as in this manner alloys can be produced of metals which will not ordinarily deposit simultaneously, as for instance, nickel and chromium. I find that if such alternate layer deposits are sufficiently thin, a metal resembling an alloy may be produced without heating. Thicker deposits can, however, be practically coalesced into an alloy by baking at their annealing temperatures, in which case if the baking be done in air, a thin, hard, glass-like oxide will also be formed upon the surface of the deposit.

The metal playing records made by the processes outlined above possess many points of superiority over the plastic composition records hitherto used in the art and made by stamping. These records are not only more faithful reproductions of the original "master," but are very light and practically unbreakable. They are, therefore, more convenient to handle and transport, and I find that they not only stand more rough usage and punishment, but also last longer in playing. A microscopic examination of the playing groove and of the needle, shows that not only does the needle wear much less than it does when used on a composition record, but that the action of the needle operates to polish or smooth out the playing grooves, thus resulting in improved playing up to certain limits, while the action of the needle on a composition record results in roughening the groove and gradually wearing it out. This microscopic examination also shows that the amount of wear of a needle on a composition record in one run alters its shape sufficiently to distort the sound groove while the wear of the needle in one run on my new metal record is almost unnoticeable and in twenty runs less than the wear of a steel needle in one run on a position record.

The present application is a continuation in part of my co-pending application, Ser. No. 306,597, filed June 25th, 1919.

What I claim is:

1. As an article of manufacture, a record having a record surface of "nickel metal." 2. As an article of manufacture, a record having a record surface of electrodeposited nickel.

3. As an article of manufacture, a master record having a record surface of "nickel metal" adapted to receive a non-adherent coating of "nickel metal" by electrodeposition. 75

4. As an article of manufacture, a master sound record comprising a main body portion of copper and a record surface portion of nickel. 80

5. As an article of manufacture, a sound record having a body portion of "nickel metal."

6. As an article of manufacture, a sound record having a body portion of "nickel metal" and an electrodeposited record surface. 85

7. As an article of manufacture, a sound record having a body portion of "nickel metal" and an electrodeposited record surface of "nickel metal." 90

8. As an article of manufacture, a sound record comprising a supporting member and a metallic record portion attached to said supporting member. 95

9. As an article of manufacture, a sound record comprising a non-metallic supporting member and a metallic record portion attached to said supporting member.

10. The process of producing sound records, which comprises electrodepositing nickel on a master record having a record surface of nickel adapted to receive a non-adherent coating of nickel by electrodeposition. 100

11. The process of producing sound records, which comprises electrodepositing a dense, substantially poreless and pitless layer of "nickel metal" on a master record having a record surface of "nickel metal" adapted to receive a non-adherent coating of "nickel metal" by electrodeposition. 110

12. The process of producing sound records, which comprises electrodepositing nickel on an electrodeposited copper master record having a record surface of nickel adapted to receive a non-adherent coating of nickel by electrodeposition. 115

13. The process of producing sound records, which comprises electrodepositing a dense, substantially poreless and pitless layer of "nickel metal" on an electrodeposited copper master record having a record surface of "nickel metal" adapted to receive a non-adherent coating of "nickel metal" by 120 electrodeposition. 125

In testimony whereof, I have signed my name to this specification this 10th day of June, 1920.

CHARLES P. MADSEN.